

1

3,788,888

### FIBER-LUBRICANT COMPOSITION

Hideo Kawanaka, Kenichi Katabe, and Seizi Kameda, Wakayama, Japan, assignors to Kao Soap Co., Ltd., Tokyo, Japan

No Drawing. Filed Apr. 16, 1971, Ser. No. 134,858  
Claims priority, application Japan, Apr. 24, 1970,

45/35,215

Int. Cl. C08j 1/44

U.S. Cl. 117—139.5 A

2 Claims

### ABSTRACT OF THE DISCLOSURE

A fiber-lubricant composition containing a copolymer of a sulfonated product of naphthalene or a naphthalene derivative with an aldehyde, or a maleic anhydride polymer or copolymer, which composition can be advantageously used as the spin finish for staple in high speed spinning of synthetic fibers.

This invention relates to a fiber-lubricant composition (or spin finish for staple) suitable for use in high speed spinning. More specifically, it relates to a basic ingredient to be incorporated in a spin finish for staple and its object is to provide a fiber-lubricant composition which can increase the fiber to fiber friction and improve the interfiber cohesion between fibers while preventing the falling-out of fibers during the drawing process.

Synthetic fibers, such as polyester fibers, acrylic fibers and polyamide fibers are used in large quantities in the spinning instead of natural fibers such as wool and cotton. In the spinning of these synthetic fibers there are various problems concerning lubricity, antistatic property, interfiber cohesion, etc. Particularly, the adaptability of the spinning process at a high speed has been a serious problem.

The spinning process of synthetic staple fibers composed mainly of polyester or dry-spun acrylic fibers cannot be conducted smoothly as compared with the case of cotton, wool or acrylic fibers made by the wet spinning process, since melt-spun polyester fibers made by the melt spinning process and acrylic fibers made by the dry spinning process have a smooth surface configuration. There occur such troubles as winding up of fibers on cylinders at the carding process and winding up of fibers on the rolls at the drawing, roving and spinning processes. Occurrence of such operational troubles is greatly influenced by not only the surface state of the fibers but also the kind of surface treating agent used for the fibers. Surface treating agents or so-called textile lubricants are generally composed of a lubricating agent and an antistatic agent. As the lubricating agent there are used animal oil, vegetable oil, mineral oil, fatty acid esters such as methyl oleate and butyl stearate, non-ionic surface active agents such as ethylene oxide adducts of fatty acids or fatty acid esters of higher or polyhydric alcohols, and anionic surface active agents such as alkyl sulfates, alkyl phosphates and fatty acid salts. As the antistatic agent there are used alkyl phosphates, alkyl sulfates, alkyl amine-ethylene oxide adducts, cationic surface active agents such as quaternary ammonium salts and alkyl betaine type amphoteric surface active agents.

In the spinning process where a property concerning the fiber to fiber friction of fibers, usually expressed by the term "interfiber cohesion" of fibers, is required, non-ionic surface active agents have been heretofore used frequently. However, with the recent development of the high speed drawing technique, when non-ionic surface active agents are used in such high speed drawing process, there occurs a trouble that fibers fall on and wind up on the drawing rolls. For this reason, alkyl phosphate salts,

2

polyoxyethylene alkyl phosphates, alkyl sulfate salts and the like are used instead of non-ionic surface active agents. However, each of these compounds does not give a high interfiber friction and the use of such compounds fails to impart a good interfiber cohesion.

More specifically, in conventional surface active agents used as spinning finishes for staple which comprise one hydrophobic group and one hydrophilic group, when the friction among fibers is increased by the use of these agents, the fiber to metal friction and the fiber to rubber friction tend to increase at the same time, which results in winding up the fibers on the rolls. If the prevention of winding up the fibers on the rolls is intended, the interfiber friction and interfiber cohesion properties of fibers should be decreased. The lowering of the interfiber cohesion property is a serious defect when labor-saving is intended by high speed carding, high speed drawing, package enlargement, etc.

Apart from the conventional idea that a surface active agent comprising one hydrophobic group and one hydrophilic group are used as the spin finish for staple or ingredients thereof, we have found that an excellent fiber-lubricant composition free of the above-mentioned defects of conventional agents can be provided by the use of specific polymers as mentioned below.

Accordingly, the object of this invention is to provide a spinning finish or a basic ingredient therefor, which can increase the degree of interfiber cohesion of fibers while reducing the fiber to metal friction and the fiber to rubber friction, whereby falling off of fibers and winding up of fibers on the rolls can be prevented in the drawing process.

The above object of this invention can be attained by using as a spinning finish for staple or a basic ingredient thereof a polymer compound which is represented by the following General Formula I or II:



wherein R and R' each is H, OH or a lower alkyl group having up to 4 carbon atoms, R'' is H or a lower alkyl group having up to 3 carbon atoms, X is a polymer constituent derived from maleic anhydride or a monomer copolymerizable with maleic acid, n designates an average degree of polymerization ranging from 3 to 10, and Me indicates hydrogen, an alkali metal, ammonium or a water-soluble, substituted ammonium cation.

Compounds of the above General Formula I may be synthesized by sulfonating naphthalene or a naphthalene derivative selected from the group consisting of alpha-naphthol, beta-naphthol, alpha-methyl-naphthalene, alpha-ethyl-naphthalene, alpha-propyl-naphthalene, alpha-butyl-naphthalene, beta-methyl-naphthalene, beta-ethyl-naphthalene, beta-propyl-naphthalene and beta-butyl-naphthalene, with a concentrated sulfuric acid at 120–170° C. and condensing the sulfonated product at 90–150° C. under acidic conditions with formaldehyde, acetaldehyde, propionaldehyde, iso-butylaldehyde or butylaldehyde.

Compounds of above General Formula II are homopolymers of maleic anhydride or copolymers of maleic anhydride with a polymerizable unsaturated compound such as ethylene, butylene, isobutylene, di-isobutylene, alpha-octene, alpha-decene, alpha-octadecene, styrene, vinyl benzene and vinyl acetate.

Compounds of the above Formulas I and II may be optionally neutralized with an alkali metal such as sodium and potassium, ammonia, an amine substituted by an organic group such as ethanolamine, diethanolamine, methylamine and dimethylamine, or a hydroxide or water-soluble salt thereof.

These fiber-lubricant compounds of this invention can exhibit their properties when they are applied to fibers in an amount of 0.05-1.0% by weight, preferably 0.1-0.5% by weight.

The treating agent of this invention may be used singly or in combination with another agent which has been used as an ingredient of a spin finish for staple, for instance, an antistatic agent.

The present invention will now be explained with reference to examples and comparative examples.

#### COMPARATIVE EXAMPLE

5 Conventional spin finish or fiber-lubricant compositions were applied to polyester filament yarns in an amount of 0.5% by weight, and the values of the interfiber friction, the fiber to metal friction and the fiber to rubber friction were determined by an Atlab friction tester. Polyester staples were treated with the same spin finish compositions and the falling off of fibers and the winding up of fibers on the rolls during the spinning process were observed. The results were as shown summarized in Table 1.

TABLE 1

| Conventional fiber-lubricant composition number | Inter fiber friction (g.) | Fiber to-           |                      | Falling off of fibers |        | Winding up of fibers on rolls |        |
|-------------------------------------------------|---------------------------|---------------------|----------------------|-----------------------|--------|-------------------------------|--------|
|                                                 |                           | Metal friction (g.) | Rubber friction (g.) | Metal                 | Rubber | Metal                         | Rubber |
| I-----                                          | 85                        | 70                  | 140                  | Middle                | Much   | 50                            | 6      |
| II-----                                         | 90                        | 100                 | 60                   | Little                | do     | 0                             | 5      |
| III-----                                        | 80                        | 110                 | 60                   | do                    | do     | 10                            | 5      |
| IV-----                                         | 90                        | 100                 | 130                  | Middle                | do     | 150                           | 10     |
| V-----                                          | 105                       | 100                 | 35                   | Little                | Little | 0                             | 0      |

As such antistatic agents, the following compounds may be preferably used:

- (1) Alkyl phosphates and polyoxyethylene alkyl phosphates (to be used mainly in the form of a sodium salt)
- (2) Polyoxyethylene alkyl sulfates (to be used mainly in the form of a sodium salt)
- (3) Fatty acid metal soaps such as potassium oleate
- (4) Non-ionic surface active agents such as polyoxyethylene alkylamines, polyoxyethylene alkylamides, polyoxyethylene alkyl ethers and polyoxyethylene alkyl esters
- (5) Betaine type amphoteric surfactants such as alkyl betaines and polyoxyalkyl betaines
- (6) Alkyl imidazoline type amphoteric surfactants
- (7) N-alkylaminopropionic acid type amphoteric surfactants

25 From the results shown in Table 1 it is seen that in the case of a fiber-lubricant composition giving a high fiber to metal friction there is a tendency that fibers wind up on metal rolls and that in the case of a composition giving a high fiber to rubber friction there is a tendency that 30 fibers wind up on rubber rolls.

#### EXAMPLE 1

Various surface active agents (agents Nos. 10 to 21 are 35 polymer compounds according to this invention and agents Nos. 1 to 9 are conventional surface active agents) were applied to polyester filament yarns in an amount of 0.5% by weight, and the values of the fiber to metal friction and the fiber to rubber friction were measured by an 40 Atlab friction tester. Results were as shown in Table 2.

TABLE 2

| Agent number | Surface active agent                      | Inter-fiber friction (g.) | Fiber to metal friction (g.) | Fiber to rubber friction (g.) |
|--------------|-------------------------------------------|---------------------------|------------------------------|-------------------------------|
| 1-----       | Potassium oleate-----                     | 68                        | 42                           | 53                            |
| 2-----       | Potassium myristyl phosphate-----         | 82                        | 52                           | 74                            |
| 3-----       | Polyoxyethylene myristyl phosphate-----   | 80                        | 100                          | 96                            |
| 4-----       | Potassium lauryl phosphate-----           | 86                        | 70                           | 38                            |
| 5-----       | Polyoxyethylene(5) oleyl ether-----       | 74                        | 90                           | 45                            |
| 6-----       | Polyoxyethylene(15) stearylamine-----     | 84                        | 140                          | 100                           |
| 7-----       | Polyoxyethylene(9) nonylphenol ether----- | 90                        | 110                          | 98                            |
| 8-----       | Polyoxyethylene(20) stearylamide-----     | 84                        | 124                          | 128                           |
| 9-----       | Sodium lauryl succinate-----              | 108                       | 146                          | 174                           |
| 10-----      |                                           | 112                       | 32                           | 24                            |
| 11-----      |                                           | 128                       | 35                           | 24                            |
| 12-----      |                                           | 126                       | 32                           | 26                            |
| 13-----      |                                           | 112                       | 82                           | 25                            |

TABLE 2—Continued

| Agent number | Surface active agent | Inter-fiber friction (g.) | Fiber to metal friction (g.) | Fiber to rubber friction (g.) |
|--------------|----------------------|---------------------------|------------------------------|-------------------------------|
| 14.....      |                      | 126                       | 45                           | 23                            |
| 15.....      |                      | 132                       | 38                           | 20                            |
| 16.....      |                      | 128                       | 37                           | 25                            |
| 17.....      |                      | 132                       | 39                           | 30                            |
| 18.....      |                      | 114                       | 30                           | 23                            |
| 19.....      |                      | 140                       | 34                           | 30                            |
| 20.....      |                      | 115                       | 30                           | 21                            |
| 21.....      |                      | 118                       | 27                           | 21                            |

(The measurement was conducted under an initial load of 15 g. and at a running yarn speed of 145 m./min.)

#### EXAMPLE 2

Mixtures of a polymer compound according to the present invention and an antistatic agent at ratios indicated below were applied to polyester staples as spin finish for staple and the spinning test was conducted. Good results shown in Table 3 were obtained.

|                                                                                       | Mixing ratio (percent by weight) |                |
|---------------------------------------------------------------------------------------|----------------------------------|----------------|
|                                                                                       | Composition I                    | Composition II |
| Di-isobutylene-maleic anhydride copolymer (average molecular weight=about 3,000)..... | 60                               | 40             |
| Potassium octyl phosphate.....                                                        | 40                               | 60             |

TABLE 3

|                                                               | Composition I     | Composition II    |
|---------------------------------------------------------------|-------------------|-------------------|
| Item:                                                         |                   |                   |
| Amount applied (percent by weight based on fiber weight)..... | 0.2               | 0.3               |
| Surface electric resistance (ohm).....                        | $3.6 \times 10^8$ | $1.4 \times 10^8$ |
| Card electrification voltage, volt.....                       | 0                 | 0                 |

TABLE 3—Continued

| Item:                                                                                                                     | Composition I | Composition II |
|---------------------------------------------------------------------------------------------------------------------------|---------------|----------------|
| Falling on carding cylinder, percent.....                                                                                 | <2            | <2             |
| Web uniformity.....                                                                                                       | Good          | Good           |
| Siliver compactness.....                                                                                                  | Good          | Good           |
| 55 Final tension on the friction tester (amount applied of spin finish composition=p.5% by weight based on fiber weight): |               |                |
| Fiber-metal friction, g.....                                                                                              | 38            | 57             |
| Fiber-fiber friction, g.....                                                                                              | 156           | 138            |
| Fiber-rubber friction, g.....                                                                                             | 41            | 40             |
| 60                                                                                                                        |               |                |

The embodiments of the invention in which an exclusive property or privilege is claimed are defined as follows:

1. Synthetic staple fiber having coated thereon from 0.05 to 1.0 percent by weight, based on the weight of staple fiber, of a polymer of the formula



wherein R and R' are H, OH or alkyl having from 1 to 4 carbon atoms, R'' is H or alkyl having from 1 to 3

carbon atoms,  $n$  is an average degree of polymerization in the range of from 3 to 10, and Me is H, alkali metal, ammonium or water-soluble substituted ammonium cation.

2. A fiber-lubricating and antistatic composition consisting essentially of from 40 to 60 percent by weight of diisobutylene-maleic anhydride copolymer and the balance is potassium octyl phosphate.

|             |         |                                |
|-------------|---------|--------------------------------|
| 2,614,984   | 10/1952 | Thomas et al. __ 117—139.5 CQ  |
| 2,289,760   | 7/1942  | Dickey et al. __ 117—139.5 CQ  |
| 2,199,989   | 5/1940  | Dickey et al. __ 117—139.5 CQ  |
| 2,676,122   | 4/1954  | McCarthy _____ 117—139.5 CQ    |
| 2,683,101   | 7/1954  | Riley et al. _____ 117—138.8 X |
| 5 2,976,186 | 3/1961  | Thompson et al. _____          |
|             |         | 117—139.5 CQ                   |
| 3,619,274   | 11/1971 | Proffitt _____ 117—138.8 F     |

## References Cited

## UNITED STATES PATENTS

|           |        |                                   |
|-----------|--------|-----------------------------------|
| 1,336,759 | 4/1920 | Schmidt _____ 260—67 S            |
| 1,848,883 | 3/1932 | Hill _____ 260—67 S               |
| 3,030,342 | 4/1962 | Tiefenthal et al. ____ 260—78.5 T |
| 2,892,736 | 6/1959 | Johnson et al. ____ 260—78.5 T 15 |

10 WILLIAM D. MARTIN, Primary Examiner

T. G. DAVIS, Assistant Examiner

U.S. Cl. X.R.

117—138.8 F, 138.8 N, 138.8 UA; 260—78.5 R